

Nov. 13, 1923.

1,473,837

J. H. DOUGLAS

FIRE KINDLER

Filed June 21, 1922

FIG. 1.



FIG. 2.



Inventor

John H. Douglas  
By A. H. Patterson

Attorney

Patented Nov. 13, 1923.

1,473,837

# UNITED STATES PATENT OFFICE.

JOHN H. DOUGLAS, OF BRADFORD, PENNSYLVANIA.

## FIRE KINDLER.

Application filed June 21, 1922. Serial No. 569,817.

To all whom it may concern:

Be it known that I, JOHN H. DOUGLAS, a citizen of the United States, residing at Bradford, in the county of McKean and 5 State of Pennsylvania, have invented certain new and useful Improvements in Fire Kindlers, of which the following is a specification, reference being had therein to the accompanying drawing.

10 This invention relates to improvements in fire kindlers and more particularly to what I have termed an absorption burner.

The object of my invention is to provide 15 a fire kindler which is so constructed as to absorb oils of different characters.

Another object of my invention is to provide a fire kindler having a novel means for assisting the oil to get into the kindler and a novel means for transporting the 20 kindler.

Another object of my invention is to provide a fire kindler constructed of several different materials in certain proportions whereby a fire kindler is provided 25 which will readily absorb oil.

Other further objects and improved results of my invention will appear in the accompanying drawings and the following description.

30 In the drawings Fig. 1 is a perspective view of my improved fire kindler.

Fig. 2 is a vertical sectional view of my improved invention.

Referring now to the drawings, 1 represents 35 my fire kindler block. This block is composed of the following materials in approximately the proportion stated, viz:

|    |                 |     |
|----|-----------------|-----|
| 40 | Sand            | 67% |
|    | Cement          | 25% |
|    | Fire brick clay | 4%  |
|    | Fire clay       | 4%  |

In addition to the above materials I add 45 a small quantity of cotton or woolen waste which is done to assist in holding the mixture together and in giving porosity to the block. It will of course be readily understood that water is used in mixing these 50 materials together. When the mixture is completed it is poured into molds to make the block into any shape or size desired.

The different sized blocks will absorb 55 different amounts of oil and I have found by experiment that a cylindrical block 4 inches high and 3 inches in diameter ab-

sorbs approximately 3 ounces of fluid and that a cylindrical block 5 inches high and 4 inches in diameter absorbs approximately 4½ ounces of fluid. A larger cylindrical 60 block 12 inches high and 6 inches in diameter will absorb approximately 16 ounces of kerosene, gasoline, crude oil or other fluid.

When the kindler block mixture is poured into a mold of the desired size 65 and shape I place in the mixture an approximately triangular shaped wire 2 which has its upper end bent into an eye 3, which extends above the block. That portion of the wire within the mixture is wrapped 70 loosely with cotton or woolen waste as appears at 4. This wire and its wrapping assist in holding the block in shape and at the same time assist the block in absorbing liquid by forming an avenue of 75 ingress for the liquid while the block is being submerged for the purpose of saturating it.

The eye 3 above the block 1 provides 80 a means whereby the block can be readily lifted from place to place by the use of a hook 5 or the like.

To use my improved lighter when the mixture is hardened and when the lighter is formed as shown in the accompanying 85 drawings, the block is placed in a can filled with kerosene, gasoline or crude oil, as desired, and left in the oil for 3 or 4 hours. At the end of this time the block has absorbed as much of the liquid as it will 90 absorb and can be removed from the can and placed upon the stove grate or other place that it is intended to build a fire. Coal, wood, or the fuel intended to be 95 burned is then placed about the kindler and a match applied to the kindler block. The kindler block will readily light because of the oil which it has absorbed and thereby start the fuel burning. The length of time that the kindler will burn of course will 100 be regulated by the size of the kindler and the amount of oil which it has absorbed.

In preparing my improved kindlers for 105 shipment they will be shipped in an unprimed condition. By this I mean that immediately upon the removal of the molded block from its mold the kindler can be shipped as desired.

From the foregoing it will be seen that I 110 have provided a cheap and efficient fire kindler which is susceptible to absorption in a

high degree and at the same time have so constructed the kindler as to provide means for lifting and moving it about.

Although I have previously stated the proportions in which the several materials composing the kindler are to be used, I wish it to be readily understood that materials could be used in different proportions than those stated, without departing from the spirit of my invention. I have found by experiment that the best results are obtained in using the materials in approximately the proportions which I have specified.

Having thus described my invention, what I claim and desire to secure by Letters Patent is:

1. As an article of manufacture, a fire kindler composed of a sand base, a binder for the sand, and a wire carried within the kindler wrapped with waste, for the purpose described.
2. As an article of manufacture, a fire kindler composed of a sand base, and a cement binder for the sand, for the purpose described.
3. As an article of manufacture, a fire kindler composed of a sand base, a binder for the sand, a wire carried within the kindler, and the wire wrapped with cotton

or woolen waste, for the purpose described. 30

4. As an article of manufacture, a fire kindler composed of a sand base, a binder for the sand, a wire within the kindler and having an extending portion without the kindler, and the wire wrapped with cotton or woolen waste, for the purpose described. 35

5. As an article of manufacture, a fire kindler composed of sand, fire brick clay, fire clay, a wire wrapped with a small quantity of cotton or woollen waste, and a binder for the materials. 40

6. As an article of manufacture, a fire kindler composed of sand, fire brick clay, fire clay, and a cement binder for the materials. 45

7. As an article of manufacture, a fire kindler composed of 67% sand, 4% fire brick clay, 4% fire clay, and a cement binder constituting 25% of the mixture. 50

8. As an article of manufacture, a fire kindler composed of 67% sand, 4% fire brick clay, 4% fire clay, a small quantity of cotton or woollen waste, 25% cement to act as a binder for the materials and waste in sufficient quantity to allow the materials to be mixed. 55

In testimony whereof I hereunto affix my signature.

JOHN H. DOUGLAS.